

May 3, 1949.

T. C. WOODMAN

2,468,908

LOOM TEMPLE

Filed Sept. 16, 1943

FIG. 1



FIG. 2



FIG. 3



T. C. WOODMAN  
INVENTOR

J. Seltzer & C. W. Johnson  
ATTORNEYS

## UNITED STATES PATENT OFFICE

2,468,908

## LOOM TEMPLE

Thomas Clifford Woodman, London, England, assignor, by mesne assignments, to Celanese Corporation of America, a corporation of Delaware

Application September 16, 1943, Serial No. 502,573  
In Great Britain September 28, 1942

1 Claim. (Cl. 139—294)

**1**  
This invention relates to artificial materials and is especially concerned with the production of resilient members that may be used in substitution for rubber in many of the applications of that substance.

According to the present invention, a resilient member comprises a shaped body of fibres that are associated by being felted or matted together, said body being partially impregnated with a film-forming material. The impregnation is partial in the sense that, except perhaps in the immediate neighbourhood of the surface, the fibres are only coated to a greater or less degree with the film-forming material, the spaces between the fibres not being completely filled up so as to embed the fibres solidly on the material; at the surface of the body, however, the film-forming material may form a skin, rendering the surface of the member impervious. The degree of partial impregnation may, and usually will diminish from the surface of the member inwards, and a core of fibres may be left within the member that is not impregnated with the film-forming material. By retaining unfilled within the member the spaces between the fibres forming the shaped body, the member thus constituted retains in a large measure the resilience of the body of fibres from which it is made, while the partial impregnation of the body, besides itself contributing to the resilience of the member, protects it against wear and disintegration. Where an impervious skin is formed and retained on the body this gives the member a smooth and impervious rubber-like surface.

The partial impregnation of the body may conveniently be effected by dipping it in a dope containing the film-forming material in solution or suspension for a period long enough to bring about the required degree of partial impregnation of the body by the dope, and then removing the volatile constituents of the dope by drying. The penetration of the body of fibres by the dope may be encouraged by subjecting the body to a vacuum before immersing it in the dope. Thus the body, or a batch thereof, may be enclosed in a vacuum chamber which is then evacuated, the dope being allowed to run into the evacuated chamber in sufficient quantity to submerge the body being treated. When a sufficient quantity has been run in, the vacuum may be released so that atmospheric pressure, or an applied super-atmospheric pressure, forces the dope into the body. The excess dope is then run off, and the body removed for drying. On drying, some shrinkage of the body may occur, which must

be allowed for in calculating the size of the body of fibres employed.

If desired, the partially impregnated body may, after drying, be dipped a second time or as many times as required so as to give added protection; in this case the layer of film-forming material deposited by the first dipping prevents the dope penetrating into the body of fibrous material in the second dipping. If necessary, having regard to the nature of the film-forming material employed, the dope may contain a plasticiser for the film-forming material to prevent the film or coating on the outside of the member from being unduly brittle.

**2**  
15. The resilient members formed in accordance with the present invention may be used in substitution for members made of rubber and the like and intended to serve as stops or buffers to absorb shock or pressure. Thus, for example, the 20 resilient members may be made in the form of door-stops and like shock-absorbing buffers, resilient gaskets, shock-absorbing mountings and vibration-absorbing pads. The smooth and impervious nature of the surface of the member is 25 of particular value where resistance to the absorption of moisture is of importance for hygienic or other reasons, e. g. in buffer pads for water-closet seats. Several examples of uses to which members formed in accordance with the present invention may be put occur in textile looms in which, for example, resilient members of suitable form may be made to serve as buffers for checking the motion of the picking sticks at the 30 end of their motion, or as the shock-absorbing pads mounted on the frogs at either side of the loom. Another application in which resilient members in accordance with the invention may be used in place of rubber is in coverings for the cloth-engaging parts of loom temples. In this 35 it may be preferable to skim off the continuous skin of film-forming material in which the surface fibres of the body of fibres are embedded, the resulting smooth matt surface acting, like rubber, to grip the edges of the fabric being woven, and to hold the fabric out to its full width.

The fibrous body that is partially impregnated for the purpose of the present invention may consist of or contain animal fibres, such as wool, 40 felted together or of artificial filaments or fibres matted together to form a shaped body, or it may be a mixture of animal and artificial or other fibres. The average density of the body before 45 impregnation may be of the order of 0.2-0.4 gram per cc. corresponding in the case of a wool felt,

## 3

to a proportion of solid fibre to voids of about 15-30%.

The mass may be shaped, to the form required in the resilient member to be produced, by any suitable means, e. g. by cutting a previously formed slab or block of matted fibres, e. g. felted wool fibres, to the required shape, or by felting the fibres together by beating or hammering in the desired form in the first instance. Where a continuous skin is required on the surface of the member, it is desirable that the body of fibres should be formed in the desired shape prior to the partial impregnation thereof, since the impregnation and drying of the body fixes the form of the body. Where a continuous skin is not required, however, resilient members may be cut from blocks or thick sheets of felted fibres, partially impregnated in the manner of the invention.

As the dope with which the shaped body of fibres is partially impregnated, solutions or suspensions having a basis of various film-forming materials may be used. Thus, for example a solution in a volatile solvent of cellulose acetate or some other thermoplastic derivative of cellulose may be employed, e. g. other cellulose esters such as cellulose propionate and cellulose butyrate, mixed esters such as cellulose acetate-propionate, cellulose acetate-butyrate or cellulose acetate-stearate, and cellulose ethers such as ethyl, benzyl and hexyl cellulose. An example of substances of this kind which may, alternatively, be applied in the form of a latex or similar aqueous suspension is a complex of ethyl cellulose with a substantial proportion, say 75 to 100% of its weight, of a plasticiser such as castor oil or tricresyl phosphate. Other film-forming materials that may be applied in the form of a solution in an organic solvent are the polymerised vinyl compounds, e. g. polyvinyl acetate, a copolymer of vinyl acetate and vinyl chloride, or a polyacrylic ester. These substances, like the ethyl cellulose complex mentioned above, have a somewhat rubbery consistency which increases the resilience arising in the product from the partial character of the impregnation. Other rubber-like bodies which may be employed, preferably in the form of an aqueous suspension or latex, are polyvinyl chloride, polyvinylidene and polyisobutylene, suitably plasticised, e. g. with tri-cresyl phosphate, or polymers of dienes including the polymers of halogenated dienes such as butadiene and chloroprene, or co-polymers thereof with mono-olefinic compounds such as styrene, acrylonitrile and isobutylene, or even rubber itself and its derivatives, it being understood that the quantity of rubber involved would be far less than in a resilient member made of solid rubber or of fibrous or other core surrounded by a thick layer of solid rubber.

The proportion of film-forming material dissolved or suspended in the dope should be such as to give a dope fluid enough to penetrate below the surface of the fibrous body to the desired extent, the body being removed from the dope before excessive impregnation has occurred. Thus the dope, and the time and conditions of its application may be such that a quantity of dope equivalent to 50-95% of the voids in the fibrous body is applied, leaving an unimpregnated core, the weight of film-forming material (including plasticiser) being, for example, from 10-25% or more of the weight of the fibres according to the density of the felt, and the proportion of the voids filled with the dope.

If desired, effect materials of various kinds may be added to the dope to produce particular effects on the surface of the members. Thus dyes, pigments, abrasive materials, fire-retardants or the like may be added in this manner. Or again, solid lubricants, such as graphite, e. g. of a particle size of 5-20 microns, or talc, may be added to facilitate internal movement in the resilient member when it is distorted. These materials, or other effect materials in the form of insoluble powders, may be added not only to the dope but, in addition or alternatively, to the body of fibrous material before impregnation. This may be done, for example, by passing a current of air, laden with the powder to be incorporated, through the body so as to carry the particles into the body. In such an operation the fibrous body may become unduly compacted, and it may be necessary to raise or loosen it in a separate subsequent operation.

The following are given by way of example of the manner in which the invention may be carried out.

## Example I

Shaped blocks of wool felt having a length of 6 1/4" and a section 3/4" square having a density of 0.38 gram per c. c. are enclosed in a vacuum chamber which is then evacuated. A quantity of dope sufficient to cover the blocks (which are prevented from floating by suitable means) is then run into the chamber, the dope having the following composition:

|                                                          |       |      |
|----------------------------------------------------------|-------|------|
| Cellulose acetate                                        | grams | 800  |
| Plasticiser (triacetin or diethyl or dimethyl phthalate) | grams | 160  |
| Acetone                                                  | ccs   | 5000 |
| Benzene                                                  | ccs   | 2800 |
| Ethyl alcohol                                            | ccs   | 2200 |
| Diacetone alcohol                                        | ccs   | 400  |

When the blocks are covered, the vacuum is released, so that atmospheric pressure forces the dope into the blocks. The blocks are then removed and drained of excess dope, and dried. The resulting blocks have an increased weight corresponding to an addition of 16% by weight of film-forming material, based on the weight of the original fibres. The blocks so formed are suitable for conversion into the cloth-engaging parts of loom temples, for which purpose they are bored for the reception of a spindle, to which they are attached by means of an adhesive having a nitrocellulose base. The blocks are then turned down to a diameter of about 1/2".

## Example II

Blocks of the kind used in Example I are impregnated in a similar manner in a dope prepared by adding a mixture of 500 ccs. of powdered graphite of a particle size of the order of 15 microns, and 250 ccs. of acetone, to each litre of a dope of the following composition:

|                   |       |      |
|-------------------|-------|------|
| Cellulose acetate | grams | 800  |
| Plasticiser       | do    | 160  |
| Acetone           | ccs   | 4900 |
| Benzene           | ccs   | 2230 |
| Ethyl alcohol     | ccs   | 2480 |
| Ethyl lactate     | ccs   | 800  |

The dope carries the graphite into the interstices of the block, and the resulting product is more resilient in character, apparently by reason of lubrication of the contacts between the fibres in the product.

The accompanying drawings show products formed in the manner described above.

Fig. 1 is a section of a pad or buffer for a water-closet seat.

Fig. 2 is a section of a rectangular block of impregnated felt, and

Fig. 3 is a section of a loom temple roller having a cloth-engaging part cut from a block similar to that shown in Fig. 2.

The legends on the drawings indicate the several features of the invention exemplified in the articles shown. Thus, Figs. 1 and 2 indicate the depth of partial impregnation of the body of felted fibres, the unimpregnated core, and the formation of an impervious skin on the surface of the article. In the article shown in Fig. 1 this skin is retained, so as to resist the absorption of moisture. In the loom temple roller shown in Fig. 3, however, a matt, gripping surface is required, and the skin formed on the block shown in Fig. 2 is cut away during the formation from the block of the cylindrical body shown in Fig. 3. Said roller is provided with a bore 1 for the reception of a spindle 2.

Having described my invention, what I desire to secure by Letters Patent is:

A resilient member having the consistency of a block of soft vulcanized rubber, said resilient member comprising a cylindrical body of matted fibres, said body of fibres being partially impregnated with a flexible film-forming material in an amount of from 10 to 25% of the weight of fibres and having a core of unimpregnated fibres,

the average density of said core being from 0.2 to 0.4 gram per c. c., said member having a bore for the reception of a spindle and suitable for employment as the cloth-engaging part of a loom temple roller.

THOMAS CLIFFORD WOODMAN.

REFERENCES CITED

The following references are of record in the file of this patent:

UNITED STATES PATENTS

| Number    | Name      | Date          |
|-----------|-----------|---------------|
| 41,073    | Johnson   | Jan. 5, 1864  |
| 889,208   | Cunniff   | June 2, 1908  |
| 987,629   | Ketcheson | Mar. 21, 1911 |
| 1,331,729 | Taylor    | Feb. 24, 1920 |
| 1,379,155 | Acheson   | May 24, 1921  |
| 1,562,382 | Taylor    | Nov. 17, 1925 |
| 1,573,982 | Macadam   | Feb. 23, 1926 |
| 1,941,769 | Ward      | Jan. 2, 1934  |
| 2,096,087 | Coolidge  | Oct. 19, 1937 |
| 2,124,330 | Pascoe    | July 19, 1938 |
| 2,159,586 | Greider   | May 23, 1939  |
| 2,208,232 | Smolak    | July 16, 1940 |
| 2,267,316 | Thompson  | Dec. 23, 1941 |
| 2,295,070 | Allen     | Sept. 8, 1942 |

FOREIGN PATENTS

| Number | Country       | Date |
|--------|---------------|------|
| 1,005  | Great Britain | 1863 |
| 2,096  | Great Britain | 1883 |